

# United States Patent Office

3,166,413

Patented Jan. 19, 1965

1

3,166,413

## TUNGSTEN-CONTAINING NICKEL-CHROMIUM ALLOYS

Stuart W. K. Shaw, Sutton Coldfield, and Reginald M. Cook, King's Heath, Birmingham, England, assignors to The International Nickel Company, Inc., New York, N.Y., a corporation of Delaware

No Drawing. Filed Feb. 4, 1963, Ser. No. 256,090  
Claims priority, application Great Britain Feb. 7, 1962  
9 Claims. (Cl. 75—171)

The present invention relates to nickel-base alloys and more specifically to nickel-base alloys suitable for use under high stress at temperatures of at least 1000° C., for example, as stator and rotor blades for gas turbine engines.

Heretofore, the art has endeavored to provide alloys suitable for use under high stress at temperatures in excess of 1000° C. in gas turbine structures. Such alloys must not only be extremely strong at temperatures in excess of 1000° C. but also must be stable at lower temperatures. Although attempts were made to provide satisfactory alloys, none, as far as we are aware, was entirely successful when carried into practice commercially on an industrial scale.

It has now been discovered that by means of a novel combination of alloying elements correlated in a special manner, alloys can be provided which exhibit an advantageous combination of mechanical characteristics.

It is an object of the present invention to provide a novel alloy having a novel combination of alloying elements.

Another object of the invention is to provide a novel cast alloy for use in precision cast turbine structures.

Other objects and advantages will become apparent from the following description.

The alloys according to the invention contain, in percent by weight, about 5% to 10% chromium, about 7% to 16% tungsten, up to about 5% molybdenum and up to about 4% niobium (the sum of the contents of tungsten, molybdenum and niobium and two-thirds of the content of chromium being from 17.5% to 20.5%), about 2% to 8% aluminum, about 0.03% to 0.3% carbon, up to about 1% zirconium and up to about 0.05% boron, the balance, apart from impurities, being nickel. The principal impurities that may be present are iron, silicon and manganese and the total amount of these elements should be as low as possible and must not exceed 3%. Preferably, the iron content does not exceed 0.5%, the silicon content 0.3% and the manganese content 0.3%.

The stress-rupture lives of the alloys at temperatures above 1000° C. fall as their chromium content increases. For the longest lives, the chromium content should not exceed 9% and, advantageously, it is from 5% to 7%. The stress rupture life also depends on the total content of tungsten, molybdenum and niobium and at a given chromium content there is an optimum value of this total at which the longest lives are obtained. In alloys containing 6% chromium, the longest lives are obtained when the total W+Mo+Nb content is about 15%. With increasing contents, the optimum total W+Mo+Nb content decreases and in alloys containing 9% chromium, it is 13%. In general, the stress rupture lives of the alloys fall sharply as the value of the expression

$$\%W + \%Mo + \%Nb + \frac{1}{3}(\%Cr)$$

is decreased below 17.5% or increased above 20.5%.

Preferably, both molybdenum and niobium are present in the alloys in amounts not exceeding 4% and 2.5%, respectively, and the tungsten content is from 9% to 14%.

The effect on the stress rupture life in long tons per square inch (t.s.i.) of varying the contents of tungsten,

2

molybdenum and niobium in a series of alloys all of which also contained 6% chromium, 6% aluminum, 0.12% carbon and 0.5% zirconium, the balance being nickel and impurities, is illustrated by the results in Table I. In this table, all the alloys except Nos. 1, 5, 6, 7 and 12 are in accordance with the invention.

Table I

| 10 | Alloy No. | Composition |             |             | Stress rupture properties at 9 t.s.i./1020° C. |                        |
|----|-----------|-------------|-------------|-------------|------------------------------------------------|------------------------|
|    |           | W, percent  | Mo, percent | Nb, percent | W+Mo+Nb + $\frac{1}{3}$ Cr, percent            | Life to rupture (Hrs.) |
| 15 | 1         | 12          | 1           | 0           | 17                                             | 54                     |
|    | 2         | 13          | 1           | 0           | 18                                             | 98                     |
|    | 3         | 14          | 1           | 0           | 19                                             | 106                    |
|    | 4         | 15          | 1           | 0           | 20                                             | 87                     |
|    | 5         | 16          | 1           | 0           | 21                                             | 67                     |
|    | 6         | 4           | 4           | 1.5         | 13.5                                           | *35                    |
| 20 | 7         | 7           | 4           | 1.5         | 16.5                                           | 62                     |
|    | 8         | 8           | 4           | 1.5         | 17.5                                           | 89                     |
|    | 9         | 9           | 4           | 1.5         | 18.5                                           | 119                    |
|    | 10        | 10          | 4           | 1.5         | 19.5                                           | 87                     |
|    | 11        | 11          | 4           | 1.5         | 20.5                                           | 77                     |
|    | 12        | 13          | 4           | 1.5         | 22.5                                           | 55                     |
|    | 13        | 15          | 0           | 0           | 19                                             | 111                    |
| 25 | 14        | 11          | 4           | 0           | 19                                             | 93                     |
|    | 15        | 14          | 0           | 0.5         | 18.5                                           | 187                    |
|    | 16        | 13          | 1           | 0.5         | 18.5                                           | 135                    |
|    | 17        | 11          | 3           | 0.5         | 18.5                                           | 94                     |
|    | 18        | 12          | 2           | 1           | 19                                             | 131                    |
|    | 19        | 11          | 3           | 1           | 19                                             | 102                    |
|    | 20        | 10          | 4           | 1           | 19                                             | 75                     |
|    | 21        | 11          | 2           | 1.5         | 18.5                                           | 127                    |
| 30 | 22        | 11          | 2           | 2.5         | 19.5                                           | 112                    |
|    | 23        | 9           | 4           | 2.5         | 19.5                                           | 78                     |
|    |           |             |             |             |                                                | 10.5                   |

\*Estimated from life at 7 t.s.i./1020° C.

Comparison of the results within the series of Alloys Nos. 1 to 5 and 6 to 12 shows how the stress rupture lives increase to a maximum and again decrease as the tungsten content is increased at two different levels of molybdenum and niobium. The results for the other alloys show that their stress rupture properties remain at a high level when the proportions of tungsten, molybdenum and niobium are varied within the limits of the invention.

The aluminum content of the alloys is important and in alloys of any given base composition, variation of the aluminum content has a marked effect on the stress rupture life. The longest lives are obtained with aluminum contents in the range 5% to 7% and alloys with aluminum contents within this range are therefore particularly suitable for gas turbine rotor blades which require the best possible stress rupture properties. At lower aluminum contents, the alloys have higher melting points and alloys with from 5% down to 3.5% or even 2% aluminum are suitable for parts such as gas turbine stator blades which require a high melting point but are less highly stressed than rotor blades.

Variation of the carbon content of the alloys within the range 0.03% to 0.3% has little effect on their stress rupture properties but preferably it is from 0.05% to 0.25%.

Zirconium and boron improve the stress rupture lives of the alloys, which preferably contain at least 0.05% zirconium, with or without boron in such an amount that the value of the expression:

$$\%Zr + 10 \times (\%B) \text{ is about } 0.2\% \text{ to } 0.7\%$$

Surprisingly, it is found that the stress rupture properties of the alloys are impaired by the presence of titanium, as is shown by the results set forth in Table II, which were obtained from a series of alloys containing, apart from titanium, 6% chromium, 3% molybdenum, 12% tungsten, 0.5% niobium, 6% aluminum, 0.12% carbon, 0.5% zirconium, balance nickel.

3  
Table II

| Ti, percent | Stress rupture properties at 9 t.s.i./1020° C. |                     |
|-------------|------------------------------------------------|---------------------|
|             | Life, Hrs.                                     | Elongation, percent |
| 0           | 113                                            | 13                  |
| 1           | 60                                             | 10                  |
| 1.5         | 50                                             | 3.9                 |
| 2.5         | 27                                             | 3.8                 |

Titanium is thus an undesirable impurity and is preferably absent. In commercial manufacture, small quantities of titanium may be present in scrap employed as part of the charge and care should be taken that any titanium introduced in this way does not exceed 0.5% of the alloy and, advantageously, it is less than 0.25%.

It is an important characteristic of the alloys that they contain no vanadium. This element seriously impairs the resistance of the alloys to oxidation at high temperatures and does not improve their stress rupture properties.

It is also important that the alloys are substantially free from cobalt, and if cobalt is present as an impurity its content should not exceed about 1%. Replacement of part of the nickel in Alloy No. 15 in Table I by 10% of cobalt was found to impair the stress rupture properties at 9 t.s.i. and 1020° C., the life to rupture being reduced from 187 hours to 119 hours and the elongation from 17.3% to 12.3%.

An alloy that is particularly suitable for use in the cast form has the composition: 6% chromium, 11% tungsten, 2% molybdenum, 1.5% niobium, 6% aluminum, 0.12% carbon, 0.1% zirconium, 0.02% boron, balance nickel and impurities. Cast specimens of this composition have been found to exhibit stress rupture lives of over 100 hours under a stress of 9 t.s.i. at 1020° C. and of 95 hours under a stress of 7 t.s.i. at 1050° C. Typical impact strengths of such specimens at 900° C. are 15-18 ft. lbs. measured on unnotched 0.45 inch-diameter test pieces. After heating for 16 hours at 980° C., the impact strength measured at 900° C. was increased to 20-27 ft. lbs.

The alloys may be air melted but are preferably melted under vacuum. Whether or not they are vacuum melted, the alloys are advantageously subjected to a vacuum refining treatment comprising holding them in the molten state under high vacuum before casting the melt. We prefer to hold the melt at a temperature of 1400°-1600° C. at not more than 100 microns pressure for a period of at least 15 minutes and, advantageously, for 60 minutes or more. The duration of the treatment depends to some extent on the purity of the ingredients of the melt, being longer when less pure ingredients are employed.

When making small castings, for example, turbine blades or stress rupture test pieces, the alloys are preferably cast under vacuum but when making large castings from a melt that has been produced or refined under vacuum, it makes little difference to the properties obtained whether casting is carried out in vacuum, inert gas or air. All the stress rupture test results given in this specification were obtained on test pieces machined from cast specimens that had been vacuum cast from vacuum melted material that had been vacuum refined for at least 15 minutes at 1500° C. under a pressure of less than 1 micron.

Articles and parts cast from the alloys may be used in the as-cast condition for high temperature service, for example, as rotor blades in gas turbine engines. If desired, the alloys may be homogenized by heating in the

temperature range 850° to 1250° C. before being put into service.

The alloys also exhibit useful stress rupture properties in the wrought form after solution heating and aging.

For use at temperatures above 1000° C. under conditions such as are encountered in gas turbine engines, involving both oxidation and sulfur attack, articles and parts made from the alloys are preferably provided with a protective coating, for example, of aluminum.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. A cast alloy consisting essentially of about 5% to 10% chromium, about 7% to 16% tungsten, up to about 5% molybdenum, up to about 4% niobium with the sum of the percentages of tungsten, molybdenum and niobium plus two-thirds the percentage of chromium being about 17.5% to 20.5%, about 2% to 8% aluminum, about 0.03% to 0.3% carbon, up to about 1% zirconium, and up to about 0.05% boron with the balance being essentially nickel.

2. An alloy as in claim 1 wherein the total of the percentages of tungsten, molybdenum and niobium is about 15%.

3. An alloy as in claim 1 wherein the chromium content is about 5% to about 9%.

4. A cast alloy consisting essentially of about 6% chromium, about 11% tungsten, about 2% molybdenum, about 1.5% niobium, about 6% aluminum, about 0.123% carbon, about 0.1% zirconium, and about 0.02% boron with the balance being essentially nickel.

5. A nickel-chromium-base alloy suitable for use in turbine structures and characterized by good stress-rupture properties at relatively high stress at temperatures of at least 1000° C., said alloy consisting essentially of about 5% to 10% chromium, about 7% to 16% tungsten, up to about 5% molybdenum, up to about 4% niobium, the sum of the percentages of tungsten, molybdenum and niobium plus two-thirds the percentage of chromium being about 17.5% to 20.5%, about 2% to 8% aluminum, about 0.03% to 0.3% carbon, up to 1% zirconium, up to 0.05% boron, up to not more than 0.5% titanium, up to not more than 1% cobalt, and the balance essentially nickel.

6. An alloy as set forth in claim 5 wherein the chromium content is about 5% to about 9%.

7. An alloy as set forth in claim 6 wherein the tungsten content is about 9% to about 14%.

8. An alloy as set forth in claim 7 wherein the molybdenum content does not exceed 4% and the niobium content does not exceed about 2.5%.

9. An alloy as set forth in claim 8 wherein the chromium content is from 5% to about 7%.

References Cited in the file of this patent

UNITED STATES PATENTS

2,575,915 Guy \_\_\_\_\_ Nov. 20, 1951  
2,920,956 Nisbet et al. \_\_\_\_\_ Jan. 12, 1960  
2,948,606 Thielemann \_\_\_\_\_ Aug. 9, 1960

FOREIGN PATENTS

853,103 Great Britain \_\_\_\_\_ Nov. 2, 1960

OTHER REFERENCES

Guy: "Nickel-Base Alloys for High Temperature Applications," Preprint of paper presented at the 30th Annual Convention of the American Society for Metals, October 25-29, 1948,